

Dec. 15, 1942.

O. LANDGRAF

2,305,172

PROCESS FOR THE CONVERSION OF LIQUID SUBSTANCES  
INTO A FINELY DIVIDED FORM

Filed May 12, 1939

2 Sheets-Sheet 1

*Fig. 2.*



*Fig. 1.*



*Fig. 3<sup>a</sup>.*



*Fig. 3<sup>b</sup>.*

*Fig. 4.*



*Fig. 5.*



*Fig. 6.*



Inventor  
Otto Landgraf,

By

Barney L. Larson

Attorney

Dec. 15, 1942.

O. LANDGRAF

2,305,172

PROCESS FOR THE CONVERSION OF LIQUID SUBSTANCES  
INTO A FINELY DIVIDED FORM

Filed May 12, 1939

2 Sheets-Sheet 2

*Fig. 8*



Inventor

Otto Landgraf

By Bailey, Stephens & Fretting

Attorneys

## UNITED STATES PATENT OFFICE

2,305,172

PROCESS FOR THE CONVERSION OF  
LIQUID SUBSTANCES INTO FINELY  
DIVIDED FORM

Otto Landgraf, Frankfort-on-the-Main, Germany, assignor, by mesne assignments, to Chemical Marketing Company Inc., New York, N. Y.

Application May 12, 1939, Serial No. 273,330  
In Germany May 5, 1938

1 Claim. (Cl. 83—91)

The present invention relates to an improved process for converting molten metals into a finely divided form.

It is an object of the present invention to provide an improved process for the comminution of molten metals with the aid of a rapidly rotating element.

In accordance with the present invention the molten metals are converted into a finely divided form by causing the molten metals to impinge upon a rapidly rotating element, such as, for example, a rapidly rotating disc, thereby subjecting it to the action of centrifugal force and subject it simultaneously to a beating action transversely to the direction of impact with the rotating element, and causing a stream of cooling liquid to impinge upon the rotating element simultaneously with such molten metal, the quantity of the cooling liquid being sufficient that it is sprayed off the rotating element simultaneously with the finely divided metal. Because of the different forces acting on the molten metal to be comminuted, such as the impact of the molten metal upon the rotating element, centrifugal action and beating action, extraordinary effects, for example, with respect to the degree of fineness of the resulting comminuted product, may be obtained with large outputs.

For carrying out the process in accordance with the present invention rotating elements may be employed which are provided with inequalities, such as elevations or depressions, so that the molten metals supplied to the elements are subjected to the desired beating action. Discs provided with beating elements such as fillets, ribs or channels, which may, for example, proceed in a radial direction or obliquely thereto, may be employed in accordance with the invention. The fillets and the like may be straight or be constructed as blades in order to throw the impinging mass and resulting particles in a certain direction. The beating elements may be continuous or interrupted and staggered relative to one another so that the mass of particles which have passed an interruption is caught by the next beating element.

The surface of the rotating elements may also be provided with different kinds of beating elements, such as teeth, knife edges and the like, so that the particles upon their passage from the center of the rotating element to the periphery thereof are thrown from one beating element against another and from the latter against another, and so on, until they are finally centrifuged off in a finely divided state.

In the disposition and construction of the beating elements care must be taken that the particles are centrifuged off the rotating element and do not collect and adhere to the beating elements.

According to one embodiment of the invention, the rotating elements are provided with openings, the edges of which exert a vigorous beating action upon the molten mass and resulting particles which enter such openings. Advantageously the rotating elements are provided with beating blades and openings.

The rotating element employed in accordance with the invention may also be so constructed that it consists, along a certain radial width only, of individual beating arms, which are disposed so close together that the expanding molten metal or the particles resulting therefrom are in all instances exposed to the beating action of at least one of such beating arms and cannot fall through the intervening spaces without being struck by such beating arms.

Several embodiments of the invention are diagrammatically illustrated in the accompanying drawings.

Fig. 1 shows a plan view of a disc-like rotating element 1, which is provided with radially disposed fillets 2.

A plan view of a rotating element illustrated in Fig. 1 is shown in Fig. 2, the fillets 3 of which, however, are disposed obliquely rather than radially. The fillets may be disposed at any distance apart, the actual distance between each fillet depending on the speed of rotation of the rotating element.

Two further arrangements of the fillets are illustrated diagrammatically in Fig. 3. On the right side of the rotating element fillets, ribs or the like which are interrupted are illustrated, further slightly displaced ribs or the like being disposed at the interruptions so that the mass of particles passing through the interruptions is caught by the rib or fillet disposed behind the same. The left side of the rotating element shown in Fig. 3 illustrates ribs or fillets 4 which are of blade-like construction.

Several cross sectional shapes of the ribs or fillets are illustrated in Fig. 4. The fillets are preferably provided with a sharp edge so that they exert a cutting action. The cross sections may be rectangular, trapezoidal or arched.

Fig. 5 shows another embodiment of a rotating element in cross section, the upper surface of which is provided with teeth, each of which is triangular in cross section.

Fig. 6 illustrates rotating element 11 in which individual openings 12 are provided.

Fig. 7 shows a cross section through the rotating element with openings. The rotating element in this case must be of such thickness that when the metal falls through the openings it must necessarily be struck by the walls of the openings so that it is subjected to a lateral impact. Elevations 13 may also be provided on the rotating element next to these openings.

Fig. 8 is a side elevation of an apparatus for carrying out the present invention with a part of the casing broken away. In this figure, 14 represents the casing which serves to collect the material being comminuted. Tubes 15 and 16 respectively represent means for feeding the molten metal to be comminuted and the cooling liquid to the rotating element 17 which is provided with the beating elements 18.

When carrying out the process in accordance with the present invention with the aid of apparatus of the type hereinbefore described, it is essential to ensure that the particles do not become fixed upon the rotating element. It has been found that such disadvantage may be overcome in an excellent manner by causing a liquid, such as water, alcohol or the like, to impinge upon the disc simultaneously with the molten metals to be comminuted. These liquids to a certain extent act as friction eliminators or lubricants and prevent any particles from adhering to and forming agglomerations on the rotating element. Consequently, in carrying out the process in accordance with the present invention, a stream of molten metal is caused to impinge against the rotating disc and simultaneously therewith a liquid, for example, water, is sprayed on the rotating disc and is sprayed off together with the metal particles produced.

In carrying out the process in accordance with the present invention, it has further proved to be essential to provide for the rapid cooling of the particles produced. This, it is found, prevents the grains formed from coarsening by re-assembly of the fine particles and the formation of agglomerations which might occur on the walls of the comminuting chamber.

It was found that the liquids employed as friction eliminators and lubricants simultaneously serve as excellent cooling media. The comminu-

tion obtained is also favorably influenced by the explosive evaporation of the liquids supplied to the rotating element.

The process in accordance with the present invention is carried out, for example, by causing a molten metal, such as fused silver-copper alloy, to impinge in a thin stream upon the rapidly rotating disc which is disposed in a closed chamber while simultaneously spraying cooling water on the disc. The molten metal impinging on the disc is torn into extremely fine particles by the centrifugal forces. The comminution obtained may be extensively regulated by regulation of the thickness of the stream of molten metal supplied, the viscosity of the molten metal and the force of the impact of the molten metal upon the rotating element. By spraying cooling water on the rotating element simultaneously with the molten metal, the comminution obtained is promoted and the disc and the particles obtained are cooled.

The resulting particles of copper-silver alloy obtained by such process may be worked up very easily, for example, by roasting, dissolving out the copper with sulfuric acid and working up the silver, whereby silver of a high degree of purity is obtained.

When comminuting alloys of the type mentioned above, the process may, for example, be regulated so that the product obtained is of such a grain size that it passes substantially completely through a sieve having at least 50 meshes per cm.<sup>2</sup>.

I claim:

33 A process for the conversion of molten substances into finely divided form, comprising causing said molten metals to impinge on a rapidly rotating surface to subject said substances to the action of centrifugal force, simultaneously subjecting said metals to a beating action by causing the metals under the action of said centrifugal force to contact with elements disposed transversely to their normal path of movement under said force and causing a stream of cooling liquid to impinge upon the rotating surface simultaneously with such molten metals, the quantity of said liquid being sufficient that it is sprayed off the surface simultaneously with the finely divided metal.